

Jan. 16, 1940.

H. S. GEORGE  
PROCESS FOR PRODUCING RAILS

2,186,966

Filed Nov. 10, 1936

FIG. 1



FIG. 4



FIG. 2



FIG. 3



INVENTOR:

Harry S. George

## UNITED STATES PATENT OFFICE

2,186,966

## PROCESS FOR PRODUCING RAILS

Harry S. George, Massapequa, N. Y.

Application November 10, 1936, Serial No. 110,045

11 Claims. (Cl. 29—169)

This invention relates to railroad rails that have their treads reenforced or built up with a layer of wear resisting alloy, and comprises improvements, in the disposition of the added metal thereon and in its final character, and also improvements in the process of applying the same. It is especially useful in building up the battered tread surfaces at rail joints. Before describing the invention in detail certain facts will be set forth pertaining to the deforming action of the wheels on the rails, together with a brief discussion of the prior art relating to the repair and reenforcement of the rails, occasioned by such action.

The tread of a new rail is crowned, but the transverse contour of a car or locomotive wheel in good condition forms a straight line having an upward slope from the flange. The rail is usually canted. As a consequence of these conditions the line of contact between the wheel and the rail tread when the latter is new lies between the center and the outside edge of the rail. This line or rather strip of contact gradually widens because of abrasion and plastic flow until, after several years of service, it occupies practically the full width of the rail head.

When and where the wheels contact the rail tread at an edge (as along a side under some circumstances, and always at the rail ends) the rate of plastic flow of the rail metal is more rapid, and projecting fins of metal are formed in a manner similar to the familiar "mushrooming" of a hammer or chisel head. This lateral deformation is accompanied by a depression of the tread below the general level and, where it occurs at rail joints, results in rough riding. The battering, which originates at the rail extremity and which is most severe in that region, is gradually extended along the rail from the end so that it is likely to extend after a time for a distance of many inches.

It is a customary operation in track maintenance to build up the battered areas at the joints by applying a coating of metal over the battered surface either by the electric or the oxy-acetylene process, so as to cover the entire battered area. The present invention will be discussed in connection with the oxy-acetylene process, but it is not restricted to that process.

I have found that a Brinell hardness of 350 on the rail tread is sufficient to prevent batter under the heaviest wheel loads, and that a somewhat lower hardness, say in the range 330-340, is sufficient to practically eliminate plastic flow under the average traffic conditions. Rails as supplied

from the mill in the as-rolled condition possess a hardness far short of that necessary to resist plastic flow, usually amounting to about 275-280 Brinell. Furthermore, the hardness of rail ends built up by former methods likewise is neither uniform nor adequate, usually ranging from 250-300.

I have also found that by depositing a strip of weld metal, restricted in width to about  $\frac{3}{4}$  to  $1\frac{1}{2}$  inches, that is to say to a width less than three-quarters of the width of the head of the rail, I am enabled, as hereinafter explained, to build up worn treads of any length and to attain a substantially uniform hardness of the deposited metal sufficient to greatly reduce and even to prevent plastic flow, without the necessity of subsequent heat treatment, the depositing operation itself being inherently of a hardening nature.

Formerly, in the case of built up treads longer than approximately three inches, the requisite hardness has not been attained throughout the deposited metal because the methods hitherto in use have been inherently softening.

By making the built up strip of metal of less width than three-quarters of the width of the rail throughout at least the major portion of its length, and such major portion being of a width which can be conveniently deposited by an operator of ordinary skill at a single pass, it is possible to cause the deposited strip to be built up continuously from end to end without objectionably reheating any portion of the deposited metal which has cooled below the critical temperature and without undue retardation of the cooling rate. By depositing the metal progressively from one end to the other of the battered surface under repair and by restricting the heat input, the deposited metal may be caused to cool naturally, and at a rate sufficient to induce a suitable hardening, and without objectionable reheating and may, therefore, be caused to have a Brinell hardness of any desired value, including any value in the range 330-350, within very close limits, say five points, by controlling such variables as the width of the strip and the rate of application, as hereinafter described.

The above discussion on hardening presupposes that the added metal as well as the rail is of suitable composition, as hereinafter explained.

In accordance with one aspect of the present invention, a repaired rail section is provided having a raised strip of hardenable metal (that is, raised with respect to the laterally adjacent battered area, but at the same general level as that of the tread) which is of not more than three-

quarters the width of the rail head throughout the major portion of its length and which stands above the laterally adjacent battered tread area to carry the load across the battered joint. Such a strip is hereinafter referred to as a causeway strip.

Such a repaired joint has the advantage of economizing repair metal since not more than three-quarters of the battered area is built up as a rule, and generally substantially less than half the battered area is built up.

Besides economizing metal, the application of a repair strip in accordance with the present invention also makes possible a corresponding economy of welding gases and a similar economy of the welder's time. Extensive operations have shown that the cost of joint repair per inch has been cut approximately in half.

Besides the advantages of economy heretofore pointed out, it may be definitely stated as a fact, based on extensive observations, that rail joints repaired by the application of causeway strips as above indicated will provide smooth riding for longer periods than any rail repaired by prior methods, unless the latter are augmented by a separate heat treatment of the repaired rail.

Other objects and advantages will hereinafter appear.

In the drawing forming part of this specification and illustrating structures embodying the present invention in a manner distinguishing them from the practices of the prior art,

Fig. 1 is a fragmentary view in end elevation illustrating certain features and principles connected with rail construction and conditions of use which will serve to facilitate an understanding of the present invention;

Fig. 2 is a plan view of a pair of abutting rail heads at a rail joint having worn tread areas at their ends built up according to former methods by a sequence of adjacent beads or strips;

Figs. 3a, 3b, 3c and 3d represent similar joints built up in accordance with various practices comprehended within the present invention; and

Fig. 4 illustrates diagrammatically the characteristic temperature changes occurring at a given point on a rail tread built up by (1) former processes, and (2) the present invention.

As a basis for understanding the present invention, the conditions imposed by the rail construction and by the traffic which the rail bears, as well as the prior art practice, will first be discussed briefly.

In Figure 1, R indicates the rail tread, W the wheel tread, C the transverse length of the contact between the rail and the wheel. (The vertical distances between the successive positions of the wheel treads are shown about twice their actual amount at the time of repair in average practice.) The parenthetical suffix (1) signifies before or soon after service, (2) after several years' service, (J) at the joint after several years' service.

In all processes of building up rail treads, metal from a welding rod is melted and deposited in a fluid puddle which is progressively extended on the tread surface suitably prepared to receive it, all by well known procedures. Usually, a layer of metal about  $\frac{1}{8}$  inch thick or less is applied. The width of the puddle is usually about  $\frac{3}{4}$  to  $1\frac{1}{2}$  inches depending upon the apparatus and skill employed. The worn tread surface on the end of a rail, at the time of building up, is usually about 8 to 14 square inches in area and, because it has heretofore been considered necessary to

cover completely the worn areas and build them up to the general level of the rest of the tread, previous methods have necessitated the application of several "beads", as the deposits are termed, adjacent to each other. (See Figure 2.) The beads have been deposited either in continuous succession, or with an intermission to permit a certain amount of cooling of the metal first applied, as in the method of my co-pending application Serial Number 688,333, now Patent No. 10,207,5810.

The chief object of my previous invention was to produce a satisfactory hardness at the extreme end-portion of a built-up tread over 3 inches in length, for I had found that, in general, where such built-up treads exceed that length, too much heat is put into the rail to admit of a sufficiently rapid rate of cooling to produce the desired hardness.

The former practice, as diagrammatically illustrated in Figure 2, causes the reheating of much of the previously deposited metal, because of the disposition of the successive beads adjacent to one another. Some parts are reheated above the critical range and, if the subsequent rate of cooling is sufficiently rapid, are given a certain amount of hardness; the major portion, however, is usually reheated to a high temperature, but somewhat below the critical range. (See Figure 4, curve 1.) Such reheating, below the critical range, is known in heat treating as drawing or tempering and has a softening effect, thereby reducing the resistance of metal so treated to abrasion and plastic deformation.

I have found that it is possible and feasible to deposit a single bead of any desired length longitudinally on a depressed rail-tread area, as at a rail joint, without reheating any part of the bead that may have cooled below the critical range; and that the width of the bead and its rate of application may be utilized to control the amount of heat put into the rail and thereby the subsequent rate of cooling and the hardness of the deposited metal. Other factors that control the hardness are the apparatus, the size of the rail, the composition of the rod and the technique of its application. In the present invention, by the proper adjustment of all these factors relative to one another, it becomes possible and feasible to impart sufficient hardness to the deposited metal to prevent plastic deformation. Compare the slopes (rate of cooling) of curves 1 and 2, Figure 4, through the critical temperature.

Among the variations in the technique of gas welding are the ways in which the coating may be hammered while hot and malleable. Such hammering is customary and universal and has two purposes, (1) to shape the coating to the contour of the rail and bring it to the general tread level, and (2) to improve the physical properties by compacting the metal, and by refining its metallographic or crystalline structure. Two methods of hammering are in common use. The first and oldest method comprises a preliminary hammering with a hand hammer followed by an operation known as "flattering". "Flattering" consists in placing on the coating a properly shaped metal shoe and hammering the latter. The second, more recent practice, comprises a preliminary hand hammering, as in the first method, followed by surface grinding, using a power driven grinding wheel.

Where "flattering" is employed, it is preferable in connection with the present invention, when the highest desirable degree of hardness is the 75

objective, to dispense with the preliminary hand hammering and to apply the flatter to successive short increments of the strip (i. e., 2 to 3 inches in length) immediately after they have been deposited. The flatter should be performed expeditiously to complete the hammering operation on each increment of coating, and permit the application of the next increment to be begun before the coating has cooled below the critical temperature.

Variations in the technique of hand hammering have been practiced formerly, but the preferred method in connection with the present invention is essentially the same as that described above for "flattering", namely, the hammering of short increments, and maintaining above the critical temperature that part of the deposits adjacent to the succeeding increment, until the deposition of the latter has been started. The purpose of the preferred techniques, whether of "flattering" or hand hammering is to prevent the reheating to a high temperature below the critical temperature, of any part of the deposit that may have cooled substantially below the critical temperature.

Where the maximum desirable hardness is not required, then departures from the preferred practices of depositing and hammering are permissible.

I have found that, satisfactorily to resist flow under the heaviest American wheel loads, the hardened strip whether heat treated or built up, should have a Brinell hardness number of at least 350, before service, the corresponding scleroscope hardness being about 50. After service, the scleroscope hardness of the surface is increased, by cold work, to about 55-58. The hardness of the cold worked layer, while not correctly indicated by the Brinell test, corresponds to a Brinell number of about 375-400. I have also found that in the alloys available and feasible for coating, and in fact in rail steel itself, a hardness greater than about 425 before service may be accompanied by an undesirable brittleness; therefore I consider the range of hardness most suitable for the purpose to be from 350 to 425 Brinell, before service, corresponding to a scleroscope hardness of 50-60. After service the most desirable scleroscope range is 55-65. An object of my invention is to provide a reenforced rail tread having a hardness throughout in the preferred range, but it is to be understood that the above discussion on hardness is for guidance and not for limiting purposes, and that the most desirable hardness may vary with circumstances as, for example, the composition of the coating.

An example of an alloy capable of possessing a hardness in the preferred range contains: C, 0.50; Cr, 0.90 to 1.10; Mn, 0.90 to 1.10; Si, 0.40 to 0.60; (all in percent by weight); and the remainder principally iron. Such an alloy is now commonly used for repairing worn rail ends, but because prior processes are inherently softening in their nature and effect, as already explained, rail ends repaired in the usual manner with this and similar alloys do not possess a uniform or sufficient hardness, but are as soft as the rail itself and often even softer (that is, in substantial portions of the built up areas).

One operator may put as much heat into the rail in making a deposit 1 inch in width as another will for a 1½ inch strip, assuming equal lengths of deposits. Consequently it is advantageous and practicable to utilize the width of the strip as well as the composition of the coat-

ing to control the hardness of a welder's product, the only requirements being that the welder shall follow instructions as to the width of the strip to be applied, shall apply it at a reasonably uniform rate, and shall be furnished with customary and standard equipment operated at the usual gas pressures.

For unusually short deposits, less than about three inches long, and where maximum speed is desired, it is advisable to employ a welding rod having a somewhat lower alloy content than that indicated above, especially in respect to the chromium and carbon, in order to guard against the possibility of an excessive cooling rate causing heat cracks in the deposit.

An advantage of limiting the width of the bead is that it reduces the heat input, thereby increasing the subsequent cooling rate and, consequently, the hardness. If the rail head were coated its full width, even though only a single bead were applied (if such were practically possible without reheating), the heat input would be so great as to materially retard the cooling rate and the resulting hardness.

As an example of the method, using a welding rod of the composition specified above, a uniform hardness of the coating amounting to 58-64 scleroscope, after service, is attained by applying a central strip 1½ inches wide at a rate of one linear inch per minute on the tread of a rail weighing in the range, 100-130 pounds per yard.

A welder of ordinary skill can apply the aforesaid coating at the stated rate, with a single burner, hand operated torch consuming oxygen and acetylene at a rate of about 80 cubic feet per hour, each.

By testing specimens of an operator's work from time to time, for any given welding rod the necessary adjustment as to strip width or, alternatively the rate of application can be readily determined and hence by a proper control of these factors the production of repaired joints coming reasonably near to the most desirable hardness can be uniformly obtained.

The technique of the coating process is important chiefly because of its effect on the composition of the deposited metal. A flame adjusted to an excess of acetylene is preferable, and the metal is preferably applied according to the technique described in my previously patented self-fluxing process of welding, (U. S. Patent No. 1,973,341) wherein the base metal preferably is maintained at a temperature several hundred degrees below its melting point while joining metal integrally thereto. Skillful operators, however, can apply the coating with a neutral flame, at the same time melting the base metal, without unduly affecting the composition of the deposited metal; but as thus practiced, there is danger on the one hand of loss of the essential elements in the rod by oxidation, and on the other hand of adding too much carbon from admixed rail metal.

An important precaution in any case is to refrain from operating too continuously with the inner cone of the flame (oxidizing in effect) buried in the molten deposit. Excessive working over the molten deposit with the flame depletes the essential hardening elements. The flame is preferably pointed almost vertically downward, but if inclined, it should be directed ahead and not backward over the already deposited metal that has started to cool.

In case the application of metal is temporarily stopped, to hammer the bead, for example, after

completing one rail end, care should be taken not to point the flame toward the finished deposit when the operation is resumed.

Although the essentials of the correct procedure for building up rail treads in accordance with the present invention have been specified above, it is neither practicable nor necessary to restrict the individual technique or minor manipulations.

The requirement that the hardness of the product shall fall within a specified range affords a ready means, not hitherto available because not applicable to former processes, of establishing a criterion of the quality of the product and controlling it, as will be understood from metallurgical considerations.

The built-up tread may be finished smooth and to the proper level by hammering or grinding or both, and the ends of the rails finished by slotting, as is customary.

The surface of the hardened strip is preferably shaped to produce a central strip thereon at a higher level than the sides, to cause the wheel to bear on the higher central strip and thereby protect the edges of the strip from concentrated loading and possible deformation. In Figure 1, S represents the central contact strip and the width thereof on the hardened strip whose sides slope to the lines on the rail at the extremities of the depression, D. The elevation of the contact strip, S, is the same as that of the rail tread intermediate of the rail ends.

When the present invention is practiced in the preferred form, that is, when the causeway strip, composed of the cited rod composition or its equivalent, is applied progressively and without the reheating of any part thereof, the resulting metallographic structure, of both the coating and the contiguous rail metal, as well as their hardness, serves to distinguish them from the products of other processes. The coating is characterized by a crystalline structure typical of metal that has been heated to its melting point and then cooled at a sufficiently rapid rate to induce a substantial hardening, while the structure throughout consists of sorbite or troostite, or a mixture thereof, without any pearlite or martensite. Even though pearlite, sorbite and troostite be considered as variations of the same structure, yet these variations are readily identified, microscopically and otherwise.

One practical advantage in the production of, say, troostite, by direct, primary cooling, rather than by first producing the hard, brittle martensite and then tempering it, is the obviation of the danger of producing heat cracks. Furthermore, the direct production of troostite is much simpler, more expeditious, cheaper, is more controllable, and results in greater uniformity, than the indirect method. In a word, the preferred method combines a controlled heat treatment with the welding operation.

Obviously, the factors which affect the structure and the hardness of the added metal, likewise influence the structure and hardness of the contiguous rail steel.

Although I have described a particular method of producing a pair of rail ends at a rail joint, having a hardened strip of metal on and longitudinal to the tread, other methods may be employed; for example, by a suitable heat treatment as described below.

As a preliminary step in my invention I prefer to grind a depression about  $\frac{1}{8}$  to  $\frac{1}{4}$  inch deep to receive a strip of weld metal of more substantial thickness than has heretofore been provided on

rail tread at joints, and this operation is necessary when utilizing the invention to reinforce new or slightly worn rails. For such rails the invention is valuable as a preventive measure, and may be conducted much more economically than after extensive wear has taken place, as heretofore. In Figure 1, D represents the depression ground in the tread.

For new rails I may use the described principle of hardening a strip of metal of limited width at the joint by heat treating a strip of the rail metal itself. The heat treated strip is preferably about  $\frac{3}{4}$  to 1 inch wide and located about the center of the tread and may extend lengthwise from 1 to 4 inches, or more, on each rail end. I have found it to be unnecessary to reinforce the ends of new rails longer than about one inch on the "leaving" rail end and about 3 inches on the "receiving" end and by so limiting the operation, whether heat treating or building up, I effect economies over previous practices, wherein the lengths of the hardened zones on each rail end are equal and unnecessarily extended.

For hardening a longitudinal strip of rail steel, as on the tread of a rail at an end thereof, I may apply heat from a row of oxy-acetylene torches, suitably supported lengthwise over the rail, spaced a suitable distance apart so that the several heated areas adjoin each other to form a continuous heated strip; after heating quickly to a bright red temperature, natural cooling is sufficient to harden the metal. As an example: to harden a rail end I may space four oxy-acetylene torches, longitudinally over the center of a rail head, with the tips 1 inch apart, that nearest the rail end being  $\frac{1}{2}$  inch therefrom; the flames, adjusted to a neutral condition, should point vertically downward, the tips of the inner cones being  $\frac{1}{8}$  inch, approximately, above the tread surface of the rail. The rate of combustion of each flame should be about 80 cubic feet per hour, each, of oxygen and acetylene. The flames should be oscillated about once a second transversely of the rail, the ends of the tips moving a distance of about  $\frac{3}{4}$  inch on each stroke. The flames should burn about 12 to 15 seconds.

For hardening a longitudinal strip of hardenable steel or alloy on the rail, a similar arrangement of torches may be used, but generally the rate of heat supply should be somewhat less and the time longer than that specified in the above example, but readily determined by trial.

Some types of electrical connections across the rail joints are brazed to the head of the rail in proximity to the rail ends. This is usually done prior to the building up process; otherwise, the brazing operation would tend to draw the temper of, or soften, the hardened strip. If for any reason the signal bonds are applied after the rail ends have been built up, the hardness can be restored by a simple treatment, applying heat in approximately the same amount and manner as when applying the coating, but preferably heating to a bright red temperature.

It should be noted that the repairing of rail joints by the strip method as herein described provides a method which does not damage signal bonds already applied whereas previous methods of repair which involve coating the entire width of the tread surface with the consequent heating of the rail metal throughout its width, frequently detaches the bonds.

The strip of deposited metal is preferably located about midway of the sides of the rail, see Fig. 3a, but it may be near or along one edge.

The strip may be applied in either direction; for example, on a rail end it may start at the "run-off", or point on the worn rail end most remote from the end edge or joint, and proceed across the joint to the other run-off; or, especially in the case of an open joint, it may be started at the end edge of one rail, proceed to the corresponding run-off, and this operation repeated in the opposite direction on the adjacent rail end. In the case of joints in which one or both ends are "chipped" extensively, it is preferable to build up the chipped ends first and then to proceed as above.

The side boundaries of the built-up strip may be straight or curved, and the width of the strip may be uniform or variable, as for example, wider at the ends than in the middle. See Figure 3d.

As a desirable modification I may widen the strip where it joins the unbattered tread, whereby a merging or transitional hardness is obtained between that of the strip and the rail at this zone.

There are advantages in having the strip extend obliquely with relation to the rail though generally in the direction of the length thereof. For example, such disposition of the strip increases the width of the contact between the wheel and the strip with relation to the actual width of the strip as measured at right angles to the side boundaries of the strip. For illustrations of this kind of construction attention is called to Figures 3b and 3c. Generally, however, where the strip is one inch wide or more, there is little advantage in the above respect.

There is also an advantage in locating the strip with respect to its position transversely of the rail to meet the special conditions imposed by various degrees of track curvature as they affect abrasion and plastic flow. For example, on curved track it is advisable in some cases to place the strip near or along the outside edge of the low rail.

The central position of the causeway strip has a decided advantage over a side position in most cases, because, among other reasons, where the wheel bears on the edge of a rail there is a much greater flow or tendency to "mushroom" for a given hardness, than where the wheel bears in the center of the rail.

While I have illustrated and described in detail certain advantageous ways of practicing the invention, it is to be understood that such illustration and description is not to be construed in a limiting sense but that it is my purpose to claim the invention broadly in whatever form its principle may be utilized.

No claim is made herein to the article produced by the present method. Claims to the repaired rail are included in my application Serial No. 189,484, filed February 9, 1938, for Repaired railroad rails, which application is a division of the present application.

I claim:

1. The process of repairing the ends of worn rail treads which comprises depositing a single continuous bead of hardenable molten metal progressively from end to end of the area under repair over an area restricted in width to not more than three-quarters of the width of the rail head and with corresponding restriction of heat input, and allowing the deposited metal which has been thus deposited and cooled below the critical temperature to be further cooled to atmospheric temperature naturally and without reheating sufficient to draw the temper of the metal.

2. The process as set forth in claim 1 in which

the metal deposited is of such character that it acquires a Brinell hardness of 330-425 when cooled in the stated manner.

3. The process as set forth in claim 1 in which the metal deposited is of such character that it acquires a resistance to plastic deformation when deposited and cooled in the stated manner substantially greater than that of the rail metal.

4. The process of repairing the ends of worn rail treads which comprises depositing hardenable metal progressively from end to end of the area under repair in the form of a single continuous longitudinal bead restricted to a width that is not greater than three quarters of the width of the rail head and that can be deposited conveniently by a torch welder at a single pass and with corresponding restriction of heat input, and causing the deposited metal which has been cooled below the critical temperature to be further cooled to atmospheric temperature without reheating, sufficient to draw the temper of the metal.

5. The process as set forth in claim 1 which further includes as a preliminary step the forming of a longitudinal depressed area in the worn surface for receiving a portion of the deposited metal.

6. The process as set forth in claim 1 in which the metal is deposited by the self-fluxing, oxy-acetylene torch method while maintaining the base metal at a temperature substantially below its melting point.

7. The process of conditioning rail ends for service which comprises heating surface tread metal above the critical temperature progressively from end to end of a longitudinally extending area restricted in width to a width not greater than three-quarters of the width of the rail head, said area being spaced inwardly from both side edges of the rail, and causing the heated metal at every point along the heated area to cool naturally to a state more resistant to plastic deformation than the original rail metal in its original state, and without subsequent reheating at any point sufficient to draw the temper of the conditioned metal.

8. A method of building up the tread surfaces of abutting rails at a rail joint, in track, the said abutting treads meeting at a depressed angle, either because of rail batter or because of angle bar wear, in which a hardenable steel welding rod is melted and deposited as a coating joined integrally with the rail, said coating being brought to the general longitudinal level of the treads of the abutting rails by a surfacing operation, to produce a smooth riding joint, said method comprising starting the building up operation at a point on one rail tread a suitable distance from the joint, depending on the extent of the depression, and depositing the rod metal as a single bead of substantially less width than the width of the rail head, and progressively extending the molten puddle in a direction substantially longitudinally of the rail, toward the junction of the rails, and continuing on the abutting rail, in the same manner and in the same direction, away from the junction, to a point a suitable distance from the junction, to make a smooth riding joint, while applying the heat employed in the operation in a manner which avoids raising the temperature of any portion of the deposited metal that has cooled below the critical or hardening temperature, thereby retaining the hardness imparted to the deposited metal.

2. The process as set forth in claim 1 in which

metal by the natural cooling effect of the underlying and adjacent rail metal.

9. The method of producing a single, longitudinally extending, hard zone of restricted width on the tread of a railroad rail, which comprises progressively heating from end to end, to a temperature above the critical range, a zone on the tread surface restricted in width to a dimension less than three-quarters of the width of the head

10. of the rail throughout at least the major portion of the length of the zone, said zone being spaced inwardly from both side edges of the rail, the rate of progress, the rate of heat input, and the amount of heat input being so adjusted in relation to one another and to the width of the zone

11. that a sharp temperature gradient is created between the zone metal and the adjacent metal of the rail head alongside of and beneath the zone metal, and the temperature gradient being so adjusted in relation to the composition of the zone metal that a zone hardness of 350-425 Brinell results upon cooling.

10. The process of repairing the ends of worn railway treads which comprises depositing a single continuous bead of hardenable molten metal progressively from end to end of the area under

25. repair over an area restricted in width to not more than three-quarters of the width of the rail head throughout at least a major portion of its length and with corresponding restriction of heat input, and allowing at least the major

portion of the length of said deposited metal, including metal deposited at the end edge of the rail, which has been deposited and cooled below the critical temperature to be further cooled to atmospheric temperature naturally and without reheating sufficient to draw the temper of the metal.

11. The method of producing a single, longitudinally extending, centrally located riding strip of restricted width on the tread of a railway rail, which comprises progressively depositing hardenable molten metal on a centrally located zone on the tread surface restricted in width to a dimension less than three-quarters of the width of the tread surface throughout at least a major portion of the length of the zone, the rate of progress, the rate of heat input, and the amount of heat input being so adjusted in relation to one another and to the width of the zone that a sharp temperature gradient is created between the zone metal and the adjacent metal of the rail head alongside of and beneath the zone metal, and the temperature gradient being so adjusted in relation to the composition of the zone metal that throughout at least the major portion of the length of said zone, including metal deposited at the end edge of the rail, a zone hardness of 330-425 Brinell results upon cooling.

HARRY S. GEORGE.